

May 20, 1941.

J. S. MARRAN

2,242,313

HEAT-RESISTING STENCIL FILM

Filed March 7, 1940

*Fig. 1.*



*Fig. 2.*



*Fig. 3.*



INVENTOR  
*John S. Marran*  
BY  
*J. R. Davis*  
ATTORNEY

## UNITED STATES PATENT OFFICE

2,242,313

## HEAT-RESISTING STENCIL FILM

John S. Marran, Stamford, Conn., assignor to  
 L. C. Smith & Corona Typewriters, Inc., Syracuse, N. Y., a corporation of New York

Application March 7, 1940, Serial No. 322,660

6 Claims. (Cl. 41—46)

This invention relates to opaque stencil sheets especially adapted for use in projecting machines such as moving-picture projectors and stereopticons.

Stencil sheets for use in motion-picture projectors or stereopticons are subjected to a high degree of concentrated heat. It is necessary therefore that the opaque coating on the sheet be heat resistant to a comparatively high degree so that the concentrated heat from the projecting lamp shall not cause a deterioration, or disintegration, of the opaque coating during the passage of the stencil sheet through the projecting machine at a normal projection speed.

One of the objects of this invention is to provide a stencil sheet with an opaque coating of such character as to be heat resistant to such a degree as to be unaffected by the heat in the projecting machine while the stencil is passing through the projecting machine at a normal speed of projection.

A further object of the invention is to provide a flexible, opaque, heat-resistant stencil sheet having a thin, tough, flexible, transparent base, preferably Cellophane, coated with an opaque coating of such character as to be removed or displaced from the base by the pressure of the type of a typewriting machine or by a stylus, or other instrument, without injury to the base, to thereby produce a clear, transparent character through which the light from the projecting machine will readily pass.

A further object of the invention is to provide an opaque coating embodying a heat-resisting or heat-reflecting metallic powder, a small portion of which powder will adhere to the Cellophane base after the opaque coating has been driven off by a typewriting machine, or other means, the said adhering portion of the heat-resisting metallic powder serving in the nature of a light filter to soften the projected light and to prevent glare on the projection screen.

In the drawing,

Fig. 1 is a view of a portion of a stencil sheet showing characters printed thereon;

Fig. 2 is a sectional view on the line 2—2 of Fig. 1; and

Fig. 3 is an enlarged sectional view of a portion of the stencil sheet.

The base 1 of the stencil may be any suitable form of thin, flexible, tough, non-absorbent and transparent material. The commercial product known as Cellophane has been found to be practical and satisfactory. The opaque coating 2 may be formed by combining any form of opaque ma-

terial, such as mineral black, a non-drying oil and a vegetable wax. With this material is combined a heat-resisting material, preferably a metallic dust. Aluminum dust or powder gives to the coating a heat-resisting and heat-reflecting quality and prevents the heat from the projection lamp affecting the oil and wax during the period of projection with the stencil moving through the projecting machine at a normal projection speed.

A satisfactory formula for the production of the opaque coating has been found to be mineral black 5%—aluminum dust or powder 34%—non-drying oil 12%—vegetable wax 49%, all by weight. The oil and wax and mineral black are ground together under suitable temperature conditions to thoroughly mix them and bring them to the desired consistency. The aluminum dust or powder is then slowly and carefully ground into the mixture until it is completely and uniformly distributed throughout the mass, and the mixture is of uniform density. This mixture is then applied to the Cellophane film base preferably to one side only, by any suitable means, preferably by a roller distributor, and the film base with the coating applied is then dried.

The proportions of the ingredients may be varied within reasonable limits without materially affecting the heat-resisting qualities of the stencil sheet. It has been found, however, that a small percentage of mineral black or equivalent opaque material is entirely satisfactory for the stencil sheet when combined with aluminum powder.

A stencil sheet produced as described may be passed through a typewriting machine and typed upon in the usual manner, the type being brought into contact with the uncoated side of the Cellophane sheet. The film, when placed in a typewriting machine, is backed by a sheet of comparatively soft paper, placed over the coated side, and the opaque coating is driven off by a single stroke of the type and adheres to the paper, thereby producing a clear outline of the typed character on the stencil base or film.

The adhesion of the opaque coating to the film must be such that any portion of the coating may be mechanically removed by writing thereon with a typewriting machine, or a stylus or other pressure instrument, thereby forming transparent or translucent characters by exposing the film base and contrasting it with the opaque coating surrounding the characters typed on the film. It is desirable that the degree of adhesion of the opaque coating to the film be such that practically all of the coating will be removed from the film by a single stroke or pressure impression.

of a type. Aluminum powder contributes materially to producing a coating which may be driven off the film base freely and sharply by a single stroke of the type of a typewriting machine, leaving the transparent film clean of opaque material and the impression sharp.

A small amount of the aluminum powder will adhere to the base film after the opaque coating has been driven off the type. This remaining small portion of the powder will serve in the nature of a filter slightly obstructing the passage of the light from the projecting machine and thereby preventing a glaring effect on the projection screen.

Bronze powder has also been found to be satisfactory as a heat resisting material. The bronze powder is mixed with the other ingredients in about the same proportion as the aluminum dust or powder, namely approximately 34% by weight.

What I claim is:

1. A heat-resisting stencil film comprising a thin, tough, flexible, transparent Cellophane base, and a coating including mineral black 5%, a non-drying oil 12%, a vegetable wax 49% and aluminum powder 34%, all by weight.

2. A heat-resisting stencil film comprising a thin, tough, flexible, transparent Cellophane base, and a coating including mineral black 5%,

15 a non-drying oil 12%, a vegetable wax 49% and metallic powder 34%, all by weight.

3. A heat-resisting stencil film comprising a thin, tough, flexible, transparent Cellophane base, and a coating including mineral black, a non-drying oil, a vegetable wax and aluminum powder, the proportion, by weight, of aluminum powder greatly exceeding the proportion, by weight, of mineral black.

10 4. A heat-resisting stencil film comprising a thin, tough, flexible, transparent base, and a coating including a powdered opaque material, oil and wax and a metallic powder, the metallic powder constituting approximately one-third, by weight, of the coating.

5. A heat-resisting stencil film comprising a thin, tough, flexible, non-absorbent, transparent base, and a coating including mineral black, a non-drying oil, a vegetable wax and aluminum powder, the aluminum powder constituting approximately 34%, by weight, of the coating.

20 6. A heat-resisting stencil film comprising a thin, tough, flexible, non-absorbent, transparent base, and a coating including mineral black, a non-drying oil, a vegetable wax and aluminum powder, the proportion of aluminum powder, by weight, greatly exceeding the proportion, by weight, of mineral black.

JOHN S. MARRAN.